

July 7, 1942.

N. HOLMSTEN

2,288,625

ABRASIVE DISK

Filed Oct. 18, 1941

Fig. 1.



Fig. 2.



Fig. 3.



Fig. 4.



INVENTOR.  
NIEL HOLMSTEN

BY *Wm. S. Pitchard*

ATTORNEY.

## UNITED STATES PATENT OFFICE

2,288,625

## ABRASIVE DISK

Nilo Holmsten, New Rochelle, N. Y.

Application October 18, 1941, Serial No. 415,507

16 Claims. (Cl. 51—195)

This invention relates to an abrasive element, and more particularly to a composite abrasive element for use on portable sanding machines.

The nature and objects of the instant invention will become clear from the following description, appended claims, and accompanying drawing forming a part of this specification and wherein:

Figure 1 is a top plan view of one form of the composite abrasive element constituting the instant invention;

Figure 2 is a section taken on the line 2—2 of Figure 1;

Figure 3 is an enlarged elevation, partly broken away, of one embodiment of a backing of the composite abrasive element; and

Figure 4 is an enlarged elevation, partly broken away, of another embodiment of a backing of the composite abrasive element.

In view of the details of construction hereafter set forth, there is provided a composite abrasive element which is characterized by a high tensile strength and a high resistance to shearing. The composite abrasive element is also sufficiently stiff so that it will normally lie flat, with the result that a smooth, vibrationless sanding operation over its entire area is obtained. In addition, the composite abrasive element is sufficiently resilient and flexible so that it will permit appreciable distortion at any point without breaking. Further, the composite abrasive element is so constructed that there will be no separation of the component parts thereof during use, either under dry or wet conditions.

In accordance with the principles of this invention, abrasive grits are adhesively secured to one surface of a fibrous sheet material and the other (opposite) surface of said fibrous sheet material is adhesively secured to a coextensive ply-wood backing. The resulting product is subjected to a treatment under controlled conditions whereby the free moisture is reduced to a minimum or even eliminated from the product. After the material has been dried, it is cut into disks of the desired shape and size. If desired, at this stage of the process the exposed surface of the ply-wood backing may be marked by printing or stamping any desired indicia, such as, for example, to identify the grit numbers and give any other desirable information. The disks are then coated on all sides thereof, as by dipping in a solution of a synthetic resin which sets upon heating to form a waterproof, heat-resistant coating. The coated disks are subjected to

an elevated temperature until the resin is converted into the insoluble, infusible state.

The dipping of the entire disk into the solution of synthetic resin seals the (cut) edges and extends over the face and backing of the disk. The method of application and the subsequent conversion of the resin provides a thin film all over the disk whereby the latter is rendered impervious to water. Because of this, the product may be used in climates of high humidity without detracting from the value and cutting efficiency thereof. The product can be used outdoors for sanding purposes, such as automobile fenders and the like, even in rainy weather.

The thin resin coating also imparts increased adhesion of the grain to the sheet material (fabric), with the result that premature flying off of the grit during operation is inhibited.

The ply-wood constituting the backing may be formed of one or more wood plies. Satisfactory results have been obtained when the backing consists of two or three-ply ply-wood. Though the ply-wood backing, when it consists of a plurality of plies, may be constructed with the grains of the plies parallel to each other, I have found that surprising and unexpected results are obtained when the ply-wood backing is constructed so that the grain of each of the plies is angularly disposed with respect to the other. The preferred angular disposition of the grain of the plies with respect to each other depends on the number of plies constituting the backing.

In that embodiment of the invention which utilizes a ply-wood backing consisting of two plies, though the plies may be disposed with respect to each other so that the grain of one ply is at any angle with respect to the other, best results are secured when the grain of one of the plies is disposed at approximately right angles to the grain of the other ply.

In that embodiment of the invention which utilizes three plies, though the plies may be so disposed that the grain of each ply is at any angle with respect to the others, best results are obtained when the three plies are so arranged that in the final ply-wood the grains of adjacent plies are disposed at an angle of approximately 60° with respect to each other.

Though a ply-wood backing made of birch is preferred, the ply-wood backing may be made of any appropriate wood. I have found that satisfactory results are secured in the two-ply construction when one ply is formed of poplar and the other of gum wood. In the three-ply embodiment, I have secured satisfactory results

when the plies are formed of birch or maple, or when two of the plies are formed of birch or maple, and the remaining ply formed of the other.

The thickness of the backing, of course, depends on the desired characteristics of flexibility, stiffness, resiliency, etc. in the final product. In the two-ply embodiment, I have found that satisfactory results are obtained when the total thickness of the ply-wood backing is from .020 to .050 inch. In the three-ply embodiment, I have found that when the total thickness of the ply-wood backing is approximately .020 to .050 inch, satisfactory results are secured.

In the production of the ply-wood backing, the selected plies are laminated together by the hot pressing method. In other words, the plies are secured together by pressure in the presence of heat through the medium of a heat-hardening resin, such as a heat-hardening phenolic resin.

Any abrasive grit may be used. Emery, silicon carbide, garnet, aluminum oxide, etc. are illustrative examples of abrasive grits which may be used. The size of the grains of the abrasive grit may vary from fine to coarse, depending on the intended use of the product.

The abrasive grit is adhesively secured to the fibrous sheet material through the medium of any well-known adhesive, such as animal hide glue.

The sheet material to which the abrasive grit and the ply-wood backing are adhesively secured may be formed of various materials. Though in the preferred form fibrous sheet material, such as paper, fabric and the like, is employed, it is to be understood that other materials, such as parchment, vulcanized fibers, impregnated materials and the like, may also be used.

The adhesive for securing the ply-wood backing to the sheet material is one which sets to form a firm, flexible bond. The bond is sufficiently strong and rigid so that it will flex and not break or separate during the intended use of the product. Animal glues or rubber adhesive compositions may be mentioned as illustrative examples of adhesives which have given satisfactory results in adhesively securing the backing of the sheet material.

In the preferred form of the invention, an aqueous solution of a phenolic formaldehyde resin is utilized for completely coating the disks. Catabond #630 resin, manufactured and sold by the Catalin Corporation, is an illustrative example of a satisfactory phenolic formaldehyde resin which may be utilized. Since the resin is water-soluble, the viscosity thereof can be modified in accordance with the grain size of the grit. It is, of course, to be understood that the final resin coating is of a thickness which does not impair the desired function of the abrasive grit in the final product.

In order to more fully explain the nature of the invention, the embodiment thereof which relates to abrasive disks of the type and nature which are secured to portable grinding heads will now be described.

Referring now to the drawing, wherein an abrasive disk of the previously-mentioned type is illustrated, and wherein like reference numerals designate like parts, the reference numeral 1 designates generally the composite abrasive disk which comprises the ply-wood backing 2 to which a sheet material (fabric) 3 is adhesively secured by means of an adhesive 4 of the type and nature previously described. On the

free surface of the fabric, an abrasive grit 5 is adhesively secured by means of an adhesive 6, also previously described.

The abrasive disk 1 is provided with a central aperture or opening 7, whereby said disk may be mounted on a grinding head. To facilitate the mounting of the abrasive disk 1 on the grinding head, there is provided a pair of diametrically opposed slits 8. As shown in the drawing, one end of each slit 8 communicates with the central opening 7, the opposite end of each slit 8 being provided with a circular hole 9 whereby, when the disk is mounted on the grinding head, the slits will not be ripped beyond their desired termini.

The abrasive disk 1 is provided with a coating 11 of a phenolic resin which extends over all of the exposed surfaces of the disk. The coating 11 not only extends over the top and bottom surfaces of the disk, but also over the entire circumferential wall of the disk and the peripheral walls of the holes 7 and 9, as well as the side walls of the slits 8.

Referring now to Figure 3, it will be noted that in the form shown therein, the backing is composed of two plies 10 and 12 adhesively secured together through the medium of the selected adhesive (not shown). It is to be noted that in this embodiment the plies 10 and 12 are so arranged and disposed with respect to each other that the grains 10' and 12' of the plies 10 and 12 respectively are at approximately right angles to each other.

In Figure 4, there is illustrated a ply-wood 35 backing formed of three plies 15, 16 and 17, the plies being adhesively secured together by means of a known adhesive (not shown). In this embodiment, it will be noted that the grain 15' of the ply 15 is disposed at an angle of approximately 60° with respect to the grain 16' of the ply 16 and that the grain 17' of ply 17 is disposed at an angle of approximately 60° with respect to the grain 16'. In other words, in the three-ply embodiment, the angularity between the grains in adjacent plies is approximately 60°.

In producing the abrasive disk element, one surface of the selected sheet material (fabric) 3, preferably of considerable length, is rendered tacky with the chosen adhesive, and the abrasive grit applied thereto. The grit-coated sheet material is dried for a time (about 1 to 2 minutes) to set the adhesive, and thereafter the chosen adhesive is applied to the grit surface and, after passing under a rubber roller whereby the quantity of adhesive is controlled and the grit surface sufficiently exposed to permit its desired function, the material is dried. Thereafter, the selected adhesive is applied to the opposite surface of the sheet material or to the top surface of the ply-wood backing (which is coextensive with the sheet material 3) to which the sheet material is to be secured, or both of said surfaces, and the materials preferably united under sufficient pressure to bring said material into intimate contact with each other. The resulting product is then dried under controlled temperature and humidity conditions until all the excessive moisture is reduced to a minimum or eliminated from the product. The preferred conditions are approximately 70° C. and a humidity of from 35%-50%. Under these conditions of temperature and humidity, I have found that satisfactory results are secured when the material is subjected thereto for at least 2 hours. Subsequently, the material is cut into disks on a power

press having a die which will stamp out the disks on a power press having a die which will stamp out the disks of the type previously described and of the desired size, shape, etc. Each individual disk at this stage of the process is provided with appropriate indicia, either by stencil, stamping, printing, etc. on the exposed surface of the ply-wood backing.

Each individual disk is then dipped into a bath containing an aqueous solution of a phenolic formaldehyde resin. After the disks have been coated as just described, they are subjected to heat (preferably in an oven) for a period of about 10 to 12 hours, at a temperature of 180°-200° C., whereby the phenolic resin is set to the waterproof, insoluble and infusible state. In the preferred form, heated air is circulated in the oven in order to insure proper and uniform drying of all parts of the disk coated with the resin.

The ply-wood backings are made by hot pressing, as previously described, it being understood that the various plies are arranged so that the grains thereof will run at the desired angles.

Since it is obvious that various changes and modifications may be made in the above description without departing from the nature or spirit thereof, this invention is not restricted thereto except as set forth in the appended claims.

I claim:

1. A composite abrasive disk element comprising a ply-wood backing, a sheet material having one surface adhesively secured to said backing, and abrasive grit adhesively secured to the other surface of said sheet material, said disk element having a coating of a waterproof resin over all the surfaces and edges thereof, said coating being of a thickness which does not impair the desired function of the grit, said disk element being sufficiently stiff so that it will lie flat and sufficiently resilient and flexible so that it will permit appreciable distortion without breaking.

2. A composite abrasive disk element comprising a ply-wood backing, a sheet material having one surface adhesively secured to said backing, and abrasive grit adhesively secured to the other surface of said sheet material, said ply-wood backing being formed of a plurality of plies so disposed with respect to each other that the grain of each ply is at an angle to the other, said disk element having a coating of a waterproof resin over all the surfaces and edges thereof, said coating being of a thickness which does not impair the desired function of the grit, said disk element being sufficiently stiff so that it will lie flat and sufficiently resilient and flexible so that it will permit appreciable distortion without breaking.

3. A composite abrasive disk element comprising a ply-wood backing, a sheet material having one surface adhesively secured to said backing, and abrasive grit adhesively secured to the other surface of said sheet material, said ply-wood backing being formed of two plies so disposed with respect to each other that the grain of one ply is at an angle of approximately 90° to the grain of the other ply, said disk element having a coating of a waterproof resin over all the surfaces and edges thereof, said coating being of a thickness which does not impair the desired function of the grit, said disk element being sufficiently stiff so that it will lie flat and sufficiently resilient and flexible so that it will permit appreciable distortion without breaking.

4. A composite abrasive disk element comprising a ply-wood backing, a sheet material having

one surface adhesively secured to said backing, and abrasive grit adhesively secured to the other surface of said sheet material, said ply-wood backing being formed of three plies so disposed

5 with respect to each other that the grains of adjacent plies are at angles of approximately 60° to each other, said disk element having a coating of a waterproof resin over all the surfaces and edges thereof, said coating being of a thickness which does not impair the desired function of the grit, said disk element being sufficiently stiff so that it will lie flat and sufficiently resilient and flexible so that it will permit appreciable distortion without breaking.

10 5. A composite abrasive disk element comprising a ply-wood backing of a thickness not in excess of approximately .050 of an inch, a sheet material formed of fabric having one surface thereof adhesively secured to one surface of said backing, and abrasive grit adhesively secured to the other surface of said sheet material, said disk element having a coating of a waterproof phenolic resin over all the surfaces and edges thereof, said coating being of a thickness which does not impair the desired function of the grit, said disk element being sufficiently stiff so that it will lie flat and sufficiently resilient and flexible so that it will permit appreciable distortion without breaking.

15 6. A composite abrasive disk element comprising a ply-wood backing of a thickness not in excess of approximately .050 of an inch, a sheet material formed of fabric having one surface thereof adhesively secured to one surface of said

20 backing, and abrasive grit adhesively secured to the other surface of said sheet material, said ply-wood backing being formed of a plurality of plies so disposed with respect to each other that the grain of each ply is at an angle to the other, said disk element having a coating of a waterproof phenolic resin over all the surfaces and edges thereof, said coating being of a thickness which does not impair the desired function of the grit, said disk element being sufficiently stiff so that it will lie flat and sufficiently resilient and flexible so that it will permit appreciable distortion without breaking.

25 7. A composite abrasive disk element comprising a ply-wood backing of a thickness not in excess of approximately .050 of an inch, a sheet material formed of fabric having one surface thereof adhesively secured to one surface of said backing, and abrasive grit adhesively secured to the other surface of said sheet material, said ply-wood backing being formed of two plies so disposed with respect to each other that the grain of one ply is at an angle of approximately 90° to the grain of the other ply, said disk element having a coating of a waterproof phenolic resin over all the surfaces and edges thereof, said coating being of a thickness which does not impair the desired function of the grit, said disk element being sufficiently stiff so that it will lie flat and sufficiently resilient and flexible so that it will permit appreciable distortion without breaking.

30 8. A composite abrasive disk element comprising a ply-wood backing of a thickness not in excess of approximately .050 of an inch, a sheet material formed of fabric having one surface thereof adhesively secured to one surface of said backing, and abrasive grit adhesively secured to the other surface of said sheet material, said disk element having a coating of a waterproof phenolic resin over all the surfaces and edges thereof, said

coating being of a thickness which does not impair the desired function of the grit, said ply-wood backing being formed of three plies so disposed with respect to each other that the grains of adjacent plies are at angles of approximately 60° to each other, said disk element being sufficiently stiff so that it will lie flat and sufficiently resilient and flexible so that it will permit appreciable distortion without breaking.

9. A composite abrasive disk element comprising a ply-wood backing, a sheet material having one surface adhesively secured to said backing, and abrasive grit adhesively secured by animal glue to the other surface of said sheet material, said disk element having substantially no free moisture and a coating of a waterproof resin over all the surfaces and edges thereof, said coating being of a thickness which does not impair the desired function of the grit, said disk element being sufficiently stiff so that it will lie flat and sufficiently resilient and flexible so that it will permit appreciable distortion without breaking.

10. A composite abrasive disk element comprising a ply-wood backing, a sheet material having one surface adhesively secured to said backing, and abrasive grit adhesively secured by animal glue to the other surface of said sheet material, said ply-wood backing being formed of a plurality of plies so disposed with respect to each other that the grain of each ply is at an angle to the other, said disk element having substantially no free moisture and a coating of a waterproof resin over all the surfaces and edges thereof, said coating being of a thickness which does not impair the desired function of the grit, said disk element being sufficiently stiff so that it will lie flat and sufficiently resilient and flexible so that it will permit appreciable distortion without breaking.

11. A composite abrasive disk element comprising a ply-wood backing, a sheet material having one surface adhesively secured to said backing, and abrasive grit adhesively secured by animal glue to the other surface of said sheet material, said ply-wood backing being formed of two plies so disposed with respect to each other that the grain of one ply is at an angle of approximately 90° to the grain of the other ply, said disk element having substantially no free moisture and a coating of a waterproof resin over all the surfaces and edges thereof, said coating being of a thickness which does not impair the desired function of the grit, said disk element being sufficiently stiff so that it will lie flat and sufficiently resilient and flexible so that it will permit appreciable distortion without breaking.

12. A composite abrasive disk element comprising a ply-wood backing, a sheet material having one surface adhesively secured to said backing, and abrasive grit adhesively secured by animal glue to the other surface of said sheet material, said ply-wood backing being formed of three plies so disposed with respect to each other that the grains of adjacent plies are at angles of approximately 60° to each other, said disk element having substantially no free moisture and a coating of a waterproof resin over all the surfaces and edges thereof, said coating being of a thickness which does not impair the desired function of the grit, said disk element being sufficiently stiff so that it will lie flat and sufficiently resilient and flexible so that it will permit appreciable distortion without breaking.

13. A composite abrasive disk element com-

prising a ply-wood backing of a thickness not in excess of approximately .050 of an inch, a sheet material formed of fabric having one surface thereof adhesively secured to one surface of said backing, and abrasive grit adhesively secured by animal glue to the other surface of said sheet material, said disk element having substantially no free moisture and a coating of a waterproof phenolic resin over all the surfaces and edges thereof, said coating being of a thickness which does not impair the desired function of the grit, said disk element being sufficiently stiff so that it will lie flat and sufficiently resilient and flexible so that it will permit appreciable distortion without breaking.

14. A composite abrasive disk element comprising a ply-wood backing of a thickness not in excess of approximately .050 of an inch, a sheet material formed of fabric having one surface thereof adhesively secured to one surface of said backing, and abrasive grit adhesively secured by animal glue to the other surface of said sheet material, said ply-wood backing being formed of a plurality of plies so disposed with respect to each other that the grain of each ply is at an angle to the other, said disk element having a substantially no free moisture and a coating of a waterproof phenolic resin over all the surfaces and edges thereof, said coating being of a thickness which does not impair the desired function of the grit, said disk element being sufficiently stiff so that it will lie flat and sufficiently resilient and flexible so that it will permit appreciable distortion without breaking.

15. A composite abrasive disk element comprising a ply-wood backing of a thickness not in excess of approximately .050 of an inch, a sheet material formed of fabric having one surface thereof adhesively secured by animal glue to one surface of said backing, and abrasive grit adhesively secured to the other surface of said sheet material, said ply-wood backing being formed of two plies so disposed with respect to each other that the grain of one ply is at an angle of approximately 90° to the grain of the other ply, said disk element having substantially no free moisture and a coating of a waterproof phenolic resin over all the surfaces and edges thereof, said coating being of a thickness which does not impair the desired function of the grit, said disk element being sufficiently stiff so that it will lie flat and sufficiently resilient and flexible so that it will permit appreciable distortion without breaking.

16. A composite abrasive disk element comprising a ply-wood backing of a thickness not in excess of approximately .050 of an inch, a sheet material formed of fabric having one surface thereof adhesively secured to one surface of said backing, and abrasive grit adhesively secured by animal glue to the other surface of said sheet material, said disk element having substantially no free moisture and a coating of a waterproof phenolic resin over all the surfaces and edges thereof, said coating being of a thickness which does not impair the desired function of the grit, said ply-wood backing being formed of three plies so disposed with respect to each other that the grains of adjacent plies are at angles of approximately 60° to each other, said disk element being sufficiently stiff so that it will lie flat and sufficiently resilient and flexible so that it will permit appreciable distortion without breaking.

CERTIFICATE OF CORRECTION.

Patent No. 2,288,625.

July 7, 1942.

NIILU HOLMSTEN.

It is hereby certified that error appears in the printed specification of the above numbered patent requiring correction as follows: Page 2, first column, line 48, for "of the sheet" read --to the sheet--; and second column, line 22, for "wellas" read --well as--; page 3, first column, lines 2 and 3, strike out "on a power press having a die which will stamp out the disks"; page 4, second column, line 26, claim 14, after "having" strike out "a"; and that the said Letters Patent should be read with this correction therein that the same may conform to the record of the case in the Patent Office.

Signed and sealed this 18th day of August, A. D. 1942.

(Seal)

Henry Van Arsdale,  
Acting Commissioner of Patents.